

## UNITED STATES PATENT OFFICE

2,112,257

METHOD OF MANUFACTURE OF SMOKELESS  
POWDER

Leavitt N. Bent, Holly Oak, Del., assignor to Hercules Powder Company, Wilmington, Del., a corporation of Delaware

No Drawing. Application January 12, 1938,  
Serial No. 184,705

10 Claims. (Cl. 52—20)

This invention relates to an improved method of manufacture of smokeless powder, and more specifically to an improved method of manufacture of colloided smokeless powder grains.

- 5 Colloided smokeless powder, often called dense smokeless powder, is usually made from nitrocellulose colloided by a volatile, or non-volatile solvent therefor, or by a mixture of volatile and non-volatile solvents. The colloided mixture of
- 10 nitrocellulose and solvent or solvents is pressed into strands, which are cut into short sections known as grains. The grains are treated for removal of solvent and moisture, dried, glazed, etc. Such colloided or dense smokeless powder may, or may not, contain nitroglycerin.
- 15 In order to manufacture a satisfactory smokeless powder, it is necessary that the solvent and moisture content of the powder, known as "residual solvent", be reduced to an amount within well defined limits for the type of powder desired.
- 20 The time necessary for the removal of the solvent or solvents, the temperature to which the powder may be subjected for solvent removal and drying, the apparatus required, and the percentage of solvent recovered, are important factors in the ultimate cost of the powder.

25 Heretofore, various methods have been used for removing the solvent from the grains of dense smokeless powder. In one process, known as water-drying, the powder grains are soaked in hot water, into which the solvent diffuses. The powder grains are removed from the water and dried in a current of hot air, to remove the adhering moisture. This process is most frequently used in the case of large grains of smokeless powder for large caliber guns.

30 The process most frequently used for drying small grains of powder for small caliber guns is known as air-drying. The cut grains, containing solvent, are exposed on shallow trays in large dry-houses to a current of warm air for a long period of time. The warm air slowly removes the solvent as a vapor, in such dilute form that economical recovery of the solvent is impossible.

35 Solvent recovery, without the complete drying of the grains of smokeless powder, has heretofore been accomplished by placing the cut grains of powder, containing solvent, in a closed container. Warm air is circulated through the powder and passes through a condenser, kept cold by suit-

able refrigeration, exterior to the powder container. The air current carries the solvent vapor to the condenser, where the solvent is condensed to a liquid form and is collected and removed for re-use. The air detrained from solvent vapor is 5 heated up to a point at which it is capable of re-absorbing more solvent and is again passed through the powder grains. This cycle may be repeated indefinitely.

40 Processes for solvent removal and drying of smokeless powder have heretofore required from three to five days and large dry-house installations. In such a process, solvent is recovered, but the powder grains must subsequently be removed from the container for final drying. Large quantities of powder are exposed to risk of fire in the dry-houses. The passage of warm air through smokeless powder grains generates static electricity, the discharge of which may ignite the powder-dust attendant to such operations.

45 The equipment of dry-houses usually consists of wooden trays for holding the powder grains during the drying process. Metal trays are undesirable, because of the possibility of friction. Wooden trays are unsatisfactory, due to the possible contamination of the powder from wood splinters. Splinters are difficult to screen from the powder, and cause trouble in the machines used for loading the smokeless powder into shells. The usual dry-houses are more or less hazardous to workmen, as it is necessary to enter them from time to time to re-arrange the trays or to fill or empty the trays. Attempts to speed up the rate of drying in such dry-houses by raising the temperature or increasing the air velocity have not 50 been successful. Such changes result in caking the grains together, in distortion of the individual grains, and in surface hardening of the grains, which closes the pores and materially retards the removal of the solvent or contained moisture.

55 I am aware that there has been proposed a method of quick drying smokeless powder containing solvent by passing through a mass of grains of such powder a current of heated steam and air. Such a process gives satisfactory results on most varieties of smokeless powder, but on certain varieties, e. g., on .30 caliber military powder, it gives higher pressures in the gun than are acceptable, as is evident from the table be-

15

20

25

30

35

40

45

50

low, where A represents a normal .30 caliber smokeless powder and B represents a similar powder dried by the accelerated steam/air method of forced drying. The results were obtained in a .30 caliber model 1906 Winchester velocity-pressure gun, using Frankford Arsenal components and 173 grain 9° boat-tail bullets.

| 10 | Powder | Charge, grains | Mean velocity, foot/seconds | Mean pressure, lbs. |
|----|--------|----------------|-----------------------------|---------------------|
|    | A----- | 49.5           | 2370                        | 46,500              |
|    | B----- | 46.0           | 2683                        | 54,800              |

15 I have found that such undesirable, or even dangerous rises in pressure, even with a slightly reduced powder charge, can be very simply avoided by accelerated drying of solvent-containing powder by an improved method, consisting in 20 forcing a current of a heated fixed gas and alcohol vapor through the powder, followed by a current of heated fixed gas, to remove the last

entire content thereof is removed by such drying treatment. With my heated air/alcohol vapor process, on the contrary, none of the inorganic, water-soluble salt components of smokeless powder are removed and lost.

5 In a typical example of the carrying out of my process, I used a smokeless powder of the following composition:

|                        | Percent |
|------------------------|---------|
| Nitrocellulose-----    | 97      |
| Diphenylamine-----     | 1       |
| Diethylphthalate-----  | 1       |
| Potassium sulfate----- | 1       |
| Total-----             | 100     |

5

To 100 parts of the above composition I added 95 parts of solvent consisting of  $\frac{2}{3}$  ether and  $\frac{1}{2}$  ethyl alcohol.

I passed heated air/alcohol mixture through 20 a body of cut grains of the above solvent-containing powder as follows:

|                                                                      | Drying                 | Alcohol used, lbs. | Temp. °C. |        | Pressure, lbs. | Time, min. | Total volatiles | Residual solvent | H <sub>2</sub> O | 25   |
|----------------------------------------------------------------------|------------------------|--------------------|-----------|--------|----------------|------------|-----------------|------------------|------------------|------|
|                                                                      |                        |                    | Inlet     | Outlet |                |            |                 |                  |                  |      |
| 30                                                                   | Alcohol and heated air |                    | 40        | 12     | 5              | 3          |                 |                  |                  | 30   |
|                                                                      |                        |                    | 40        | 20     | 5              | 12         |                 |                  |                  |      |
|                                                                      |                        |                    | 40        | 44     | 5              | 15         |                 |                  |                  |      |
|                                                                      |                        |                    | 40        | 51     | 5              | 15         |                 |                  |                  |      |
|                                                                      |                        |                    | 40        | 52     | 5              | 15         |                 |                  |                  |      |
|                                                                      |                        |                    | 41        | 55     | 5              | 30         |                 |                  |                  |      |
|                                                                      |                        |                    | 38        | 52     | 5              | 30         |                 |                  |                  |      |
|                                                                      |                        |                    | 39        | 55     | 5              | 240        |                 |                  |                  |      |
|                                                                      |                        |                    | 40        | 56     | 5              | 60         |                 |                  |                  |      |
|                                                                      |                        |                    | 40        | 58     | 5              | 120        |                 |                  |                  |      |
| 35                                                                   |                        |                    | 40        | 58     | 5              | 60         |                 |                  |                  | 35   |
|                                                                      |                        |                    | 40        | 58     | 5              | 120        |                 |                  |                  |      |
|                                                                      |                        |                    | 40        | 58     | 5              | 120        |                 |                  |                  |      |
|                                                                      |                        |                    | 40        | 58     | 5              | 120        |                 |                  |                  |      |
|                                                                      |                        |                    | 40        | 59     | 5              | 120        |                 |                  |                  |      |
|                                                                      |                        |                    | 40        | 59     | 5              | 120        |                 |                  |                  |      |
|                                                                      |                        |                    | 40        | 59     | 5              | 120        |                 |                  |                  |      |
|                                                                      |                        |                    | 40        | 59     | 5              | 240        |                 |                  |                  |      |
|                                                                      |                        |                    | 54.34     |        |                |            | 24 hrs.         | 3.81             | 2.50             | 1.31 |
|                                                                      |                        |                    |           |        |                |            |                 |                  |                  |      |
| 45                                                                   | Heated air only        |                    | 55        | 52½    | 5              | 15'        |                 |                  |                  | 45   |
|                                                                      |                        |                    | 57        | 54     | 5              | 105'       |                 |                  |                  |      |
| Upon completion of the treatment the smokeless powder contained----- |                        |                    |           |        |                |            | Total volatiles | Residual solvent | H <sub>2</sub> O |      |
|                                                                      |                        |                    |           |        |                |            | 3.52            | 2.38             | 1.14             |      |

50 traces of alcohol from the powder. As fixed gas I may use air, nitrogen, carbon dioxide, and the like. As alcohol, to produce the vapor, I may use ethyl, butyl, propyl, secondary amyl, tertiary amyl, iso-butyl, secondary butyl, and iso-propyl alcohols, but not methyl alcohol, because of its solvent action on the nitrocellulose of the powder grain. I believe that my use of alcohol vapor minimizes the surface hardening of solvent-containing powders which occurs to some extent when such powders are treated by a current of 60 heated air and steam. The surfaces of the powder grains thus remaining soft, escape of the solvent from the interior of the powder grain is 65 facilitated.

A further advantage of my improved heated air/alcohol vapor process over the heated air/steam process lies in the fact that when using the latter process there is considerable dissolving action of the salt constituents, e. g., potassium or barium nitrates, by the water present. In all cases of use of the accelerated steam/air treatment a considerable proportion of the barium or potassium nitrate is lost, and in the case 75 of a powder containing potassium sulfate, the

This powder (A) was tested in a .30 caliber 1906 Winchester velocity/pressure gun, using Frankford Arsenal components and 173 grain 9° boat-tail bullets, in comparison with a normal powder (B). The results were as follows:

| Powder | Charge, grains | Mean velocity, foot/seconds | Mean pressure, lbs. |
|--------|----------------|-----------------------------|---------------------|
| A----- | 49.5           | 2,663                       | 49,100              |
| B----- | 49.5           | 2,654                       | 50,100              |

50

Thus my heated air/alcohol process of accelerated drying of smokeless powder avoids the production of high breech pressures in rifles.

65 In a further example of the carrying out of my process, I used a pyro .30 caliber powder, of the following composition:

|                        | Percent |
|------------------------|---------|
| Nitrocellulose-----    | 97      |
| Diphenylamine-----     | 1       |
| Diethylphthalate-----  | 1       |
| Potassium sulfate----- | 1       |
| Total-----             | 100     |

65

75

To 100 parts of the above composition I added 95 parts of solvent consisting of  $\frac{2}{3}$  ether and  $\frac{1}{3}$  ethyl alcohol.

I passed heated air/isopropyl alcohol mixture 5 through a body of cut grains of the above solvent-containing powder as follows:

my application, Serial No. 73,095, filed by me April 7, 1936.

What I claim and desire to protect by Letters Patent is:

1. In a method of removing solvent from 5 smokeless powder, the step comprising subject-

| 10                                                                     | *<br>Alcohol used, lbs. | Temp. ° C. |        | Pres-<br>sure,<br>lbs. | Time,<br>min. | H <sub>2</sub> O | Total<br>volatile,<br>percent | 10 |
|------------------------------------------------------------------------|-------------------------|------------|--------|------------------------|---------------|------------------|-------------------------------|----|
|                                                                        |                         | Inlet      | Outlet |                        |               |                  |                               |    |
| Heated air and alcohol.                                                |                         |            |        |                        |               |                  |                               |    |
| Do.                                                                    |                         | 17         | 40     | 5                      | 15            |                  |                               |    |
| Do.                                                                    |                         | 36         | 38     | 5                      | 15            |                  |                               |    |
| Do.                                                                    |                         | 46         | 39     | 5                      | 15            |                  |                               |    |
| Do.                                                                    |                         | 48         | 39     | 5                      | 15            |                  |                               |    |
| Do.                                                                    |                         | 49         | 39     | 5                      | 60            |                  |                               |    |
| Do.                                                                    |                         | 48         | 38     | 5                      | 180           |                  |                               |    |
| Do.                                                                    |                         | 48         | 38     | 5                      | 120           |                  |                               |    |
| Do.                                                                    |                         | 44         | 38     | 5                      | 120           |                  |                               |    |
| Do.                                                                    |                         | 40         | 38     | 5                      | 120           |                  |                               |    |
| Do.                                                                    |                         | 45         | 42     | 5                      | 120           |                  |                               |    |
| Do.                                                                    |                         | 45         | 42     | 5                      | 120           |                  |                               |    |
| Do.                                                                    |                         | 45         | 42     | 5                      | 120           |                  |                               |    |
| Do.                                                                    | 23 lbs.                 | 41         | 42     | 5                      | 120           |                  |                               |    |
| Heated air only.                                                       |                         | 58         | 64     | 5                      | 60            | H <sub>2</sub> O | Total<br>volatile,<br>percent | 25 |
| Upon completion of the above treatment the smokeless powder contained. |                         |            |        |                        |               | 1.45             | 4.51                          |    |

30 A further advantage of my improved drying process is that it allows the use of an excess of deterrent solution on the powder grains in the coating operation, with subsequent recovery of the solvent, instead of economizing in deterrent solution by using only sufficient of the deterrent 35 solution to wet the grains of powder, as has been past practice, where solvent recovery in the coating operation was impractical. In the use of an excess of deterrent solution, the entire mass of smokeless powder grains and deterrent solution 40 is placed in the drier used in my improved process, and a mixture of alcohol vapor and air at a temperature in accordance with the examples hereinbefore stated, and for a time as hereinbefore stated, is passed through the powder 45 until substantially all the powder solvent and deterrent solvent are removed, the powder then being dried by a current of warm air as described.

I do not limit my process to the treatment of any particular variety of smokeless powder, and 50 I may use my process in the drying of single or double base powders of any size or shape of granulation. The time taken by my drying treatment will naturally vary with the size or shape of the powder grain, since the larger grains will 55 require a longer time for removal of solvent than will the finer grains. I do not limit my temperatures to those shown in the examples, since I may wish to subject certain powders to a longer time of treatment at somewhat lower temperatures, and other powders to a shorter treatment 60 at somewhat higher temperatures. I may treat by my improved process the so-called deterred or progressive burning powders, i. e., those coated with a deterrent, for example dinitrotoluol, diethylphthalate, and the like.

My improved process for removal of solvent may be carried out in any suitable form or apparatus in which undried powder grains are subjected to a current of air and water vapor 70 or steam. Such apparatus may consist of a column containing the powder, a tank, a box, or any container through which can be passed the alcohol/air current which accomplishes the drying.

75 This application is a continuation-in-part of

ing smokeless powder to the action of a current of a fixed gas and a vapor of an alcohol which is 30 a non-solvent for the smokeless powder from the group consisting of ethyl, butyl, propyl, secondary amyl, tertiary amyl, isobutyl, secondary butyl, and isopropyl alcohols.

2. In a method of removing solvent from 35 smokeless powder, the step comprising subjecting smokeless powder to the action of a heated current of a fixed gas and a vapor of an alcohol which is a non-solvent for the smokeless powder from the group consisting of ethyl, butyl, propyl, 40 secondary amyl, tertiary amyl, isobutyl, secondary butyl, and isopropyl alcohols.

3. In a method of removing solvent from 45 smokeless powder, the step comprising subjecting smokeless powder to the action of a current of air and a vapor of an alcohol which is a non-solvent for smokeless powder from the group consisting of ethyl, butyl, propyl, secondary amyl, tertiary amyl, iso-butyl, secondary butyl, and isopropyl alcohols.

4. In a method of removing solvent from 55 smokeless powder, the step comprising subjecting smokeless powder to the action of a current of nitrogen and a vapor of an alcohol from the group consisting of ethyl, butyl, propyl, secondary amyl, tertiary amyl, isobutyl, secondary butyl, and isopropyl alcohols.

5. In a method of removing solvent from 60 smokeless powder, the step comprising subjecting smokeless powder to the action of a current of carbon dioxide and a vapor of an alcohol from the group consisting of ethyl, butyl, propyl, secondary amyl, tertiary amyl, isobutyl, secondary butyl, and isopropyl alcohols.

6. In a method of removing solvent from 65 smokeless powder, the step comprising subjecting smokeless powder containing water-soluble salts to the action of a current of a fixed gas and a vapor of an alcohol, which is a non-solvent for the smokeless powder, from the group consisting of ethyl, butyl, propyl, secondary amyl, tertiary amyl, isobutyl, secondary butyl and isopropyl alcohols.

7. In a method of removing solvent from 70 smokeless powder, the step comprising subject-

- ing smokeless powder to the action of a mixture of a fixed gas and a vapor of an alcohol which is a non-solvent for the smokeless powder, from the group consisting of ethyl, butyl, propyl, secondary amyl, tertiary amyl, isobutyl, secondary butyl and isopropyl alcohols, said mixed gas and alcohol vapor being heated to about 40° C.
3. In a method of removing solvent from smokeless powder, the step comprising subjecting smokeless powder containing nitrocellulose, diphenylamine, diethylphthalate, and potassium sulfate to the action of a current of a fixed gas and a vapor of an alcohol which is a non-solvent for the smokeless powder, from the group consisting of ethyl, butyl, propyl, secondary amyl, tertiary amyl, isobutyl, secondary butyl and isopropyl alcohols.
- 10
- 15

9. In a method of removing solvent from smokeless powder, the step comprising subjecting progressive burning smokeless powder to the action of a current of a fixed gas and a vapor of an alcohol which is a non-solvent for the smokeless powder, from the group consisting of ethyl, butyl, propyl, secondary amyl, tertiary amyl, isobutyl, secondary butyl, and isopropyl alcohols.

10. In a method of removing solvent from smokeless powder, the step comprising subjecting smokeless powder to the action of a heated current of air and ethyl alcohol vapor.

LEAVITT N. BENT. 15